

J. L. MILTON.  
METHOD OF MAKING ELECTRIC COILS.  
APPLICATION FILED FEB. 7, 1913.

1,326,366.

Patented Dec. 30, 1919.

2 SHEETS—SHEET 1.



Fig. 1.

Fig. 3.

Fig. 2.



Fig. 4.



Fig. 5.

Witnesses.  
J. P. McDermott Jr.  
C. F. Corkline

Inventor.

John Lewis Milton

J. L. MILTON,  
METHOD OF MAKING ELECTRIC COILS,  
APPLICATION FILED FEB. 7, 1913.

1,326,366.

Patented Dec. 30, 1919.  
2 SHEETS—SHEET 2.



Fig. 6.

Witnesses  
F. P. McDermott, Jr.  
Q. F. Conklin

Inventor  
John Lewis Milton

# UNITED STATES PATENT OFFICE.

JOHN LEWIS MILTON, OF LOUISVILLE, KENTUCKY, ASSIGNOR TO MOTOR IGNITION & DEVICES COMPANY, A CORPORATION OF WEST VIRGINIA.

## METHOD OF MAKING ELECTRIC COILS.

1,326,366.

Specification of Letters Patent. Patented Dec. 30, 1919.

Application filed February 7, 1913. Serial No. 746,933.

*To all whom it may concern:*

Be it known that I, JOHN L. MILTON, a citizen of the United States, residing at Louisville, in the county of Jefferson and State of Kentucky, have invented a certain new and useful Improvement in Methods of Making Electric Coils, of which the following is a full, clear, concise, and exact description, reference being had to the accompanying drawings, forming a part of this specification.

My invention relates to electrical coils and particularly to the process of forming them.

It was my aim in connection with the development of a high-tension ignition system for internal combustion engines, and particularly those used on automobiles, to make an induction coil of the Tesla type,—that is, a coil having a secondary winding of wire over which is wound a primary winding of coarser wire in which there is no iron core.

It was my object to develop a coil of this general type which might be attached directly to each of the spark plugs of a multi-cylinder engine. This meant necessarily that the coil would be subjected to a high temperature, due to its proximity to the cylinder of the engine. It would also be subjected to oil and grease and generally to very severe conditions of use.

Ordinarily, coils used in ignition work are impregnated with wax to establish and maintain the very high degree of insulation necessary. Subjected to the use to which I proposed to put my coils, however, the wax would soon melt and the coil would be destroyed. I decided, therefore, if possible, to make a coil in which the several layers of wire and the several conductors of each layer would be insulated from one another by a material such as bakelite or condensite which would withstand the high degree of heat and the oil and grease to which the coil would be subjected.

I have seen a great many coils wound and put into molds with bakelite and condensite subjected to the usual process of applying heat and pressure which formed the bakelite or condensite as a shell surrounding the coil. These experiments prove that the bakelite or condensite would not penetrate the interstices very far below the surface of the coil and it has also been found that the great pressure necessary for such processes has

generally destroyed the insulation on the wires by pressure or pushed the terminals or their connections out of place and generally breaking them.

It was my aim to construct a coil with all the interstices between the conductors completely filled with materials such as bakelite or condensite and as part of same process cover the coil with a similar material. I shall describe this process and the various details of my invention in connection with the accompanying drawings, in which,

Figure 1 is a section of a coil wound with the insulating material between the wires prior to impregnation. Fig. 2 is a cross-section of the same coil after impregnation. Fig. 3 is a view, one-half of which shows Fig. 1 and the other half of which shows Fig. 2. Fig. 4 shows a completed coil in commercial form and size, (smaller scale than Figs. 1, 2 and 3), mounted on a spark plug. A petticoat has been added to the coil. Fig. 5 shows the complete coil in the mold after the process is completed. Fig. 6 is a bottom view of the complete coil.

Like reference marks are applied to the same parts throughout the various figures.

Now, describing the process in detail, and in the best manner in which it may be carried out so far as I am aware. I shall first refer to Fig. 1 which shows a hub, 1, or core of bakelite or vulcanized fiber. Upon the hub 1, I first wind a layer of cotton-covered magnet wire of relatively small cross-section, next is laid a layer of porous or absorbing material, 2, such as cloth or paper. Alternate layers of wire, 3, and of absorbing material, 2, are laid up until the necessary turns of wire have been wound. The terminals 4-4 are then secured to the wire for electrical connection and are next held in place on the wound coil by binding threads or similar method. The coil completed thus far, as shown in Figs. 1 and 3, is put into an oven to be dried at a temperature of approximately 100° C, for at least three hours. While the coils are still hot they are placed in an impregnating chamber and the air quickly exhausted to about a twenty-eight inch vacuum; coils are immediately flooded with a bakelite or condensite varnish and air pressure of from 60 to 100 pounds per square inch applied. This pressure should be maintained for some three hours, and

during this period the pressure is released for a few minutes and then again applied.

The coils are then removed from the impregnating chamber and drained. Next they are put into a bake oven with temperature at about 75° C. for two or three hours, after which time the coils are again returned to the impregnating chamber for a repetition of the above vacuum process. When they have been removed from the tank and drained and then put into the oven for baking for two to three hours at 75° C., the temperature is increased to 120° C. and baked for some twelve or fifteen hours.

The coils, having reached this stage of the process, are illustrated in Fig. 3. This shows the bakelite or condensite completely filling the interstices of the winding and also serving to hold the terminals in place. The wires of the coil are now completely embedded in solid bakelite or condensite, as the case may be, which is now no longer susceptible of changing its form from the subsequent molding process. The coil having advanced this far is placed in the mold 10 of Fig. 6, together with the pre-determined quantities of bakelite or condensite. The coil 6 is guided into its correct position, as the mold closes, by the pilot pin 11, which fits into the recess 7 of the hub 1. Similar guide pins, not shown in the drawings, fit into terminals 4—4 of the coil. It will be noted that these terminals and guide pins are designed so as to permit the coil to adjust itself in its vertical movement into final position, which is incident to the process of molding. I have experienced great difficulty with other types of terminals and therefore wish to direct attention to this feature of having the terminals placed parallel with the axis of the coil. It must be noted that the plunger 12 of the mold, in its first position before applying the heat and pressure, extends above the mold casing 10<sup>a</sup>, in order to make room for the coil and the loose and unshaped insulating material. The heat softens the latter and the pressure forces it into its final shape, all being done by the well known process. The guide pins 13—13 of the mold register with holes 14—14 to govern the register of the complete mold. At the completion of the molding process the mold can be taken apart and the complete coil removed. The pressure applied by the mold I sometimes term "mechanical pressure" to distinguish it from the pressure produced by compressed air.

Particular attention is directed to the fact that the above mentioned process of impregnating and handling the coil and subsequently molding the bakelite or condensite avoids all the serious trouble heretofore incident to molding coils of such substances as bakelite or condensite.

The extension 8 to the coil 9, shown in

Figs. 4 and 5 is molded integral with the coil to provide protection to the spark plug insulation from dirt, water and oil.

The scope of my invention is indicated only by the appended claims in which I state the invention which I desire to secure by Letters Patent.

I claim as my invention:

1. A process for making electric coils, including winding alternately a layer of insulation and a layer of wire, impregnating the same with liquid bakelite or the like, baking and molding thereto additional bakelite or the like under heat and pressure. 75

2. A process for making electric coils including making a coil having layers of conducting material separated by layers of insulation, impregnating the same with bakelite or the like, and applying thereto additional bakelite or the like by molding under 85 the action of pressure.

3. A process for making electric coils including making a coil having layers of wire separated by layers of porous insulation, impregnating the same with liquid bakelite 90 or the like, baking same and applying thereto additional bakelite or the like by molding under the action of heat and pressure.

4. A process for making electric coils which includes making a coil having layers 95 of conductors separated by layers of insulation, impregnating same with liquid bakelite or the like, baking same, again impregnating same with liquid bakelite or the like, again baking same and molding additional 100 bakelite or the like thereto under the action of heat and pressure.

5. A process for making electric coils, including alternately winding a layer of insulation and a layer conducting material, impregnating the same with liquid bakelite or the like, baking same, surrounding the same with bakelite and subjecting the same to heat and mechanical pressure. 105

6. The method of treating an electrical 110 coil which comprises surrounding the turns and filling the interstices of the coil by impregnation and hardening with an insulating material capable when hardened of withstanding excessive pressure and molding 115 around the coil under pressure similar insulating material and hardening the same.

7. The method of treating an electrical coil which comprises impregnating the coil with a liquid insulating material and hardening the same so as to surround the turns or windings and fill the interstices of the coil with hardened insulating material capable of preventing distortion of the turns or windings under excessive pressure, and then 120 molding around the coil under pressure similar insulating material in plastic form and hardening the same.

8. The method of treating an electrical coil which comprises thoroughly impregnat- 130

ing the coil with bakelite or condensite or similar material in substantially liquid form and subsequently molding around the coil under pressure similar material in plastic form.

9. As an article of manufacture, an electrical coil having its individual turns in-

cased in a substantially solid mass of bakelite or the like and covered or surrounded with a molded casing of similar material.

JOHN LEWIS MILTON.

Witnesses:

F. P. McDERMOTT, Jr.,  
O. F. CONKLIN.